

(Model.)

J. M. DENNIS.  
Brush.

No. 240,103.

Patented April 12, 1881.

Fig. 1.



Fig. 2.



WITNESSES:

Francis McArdle.  
C. Sedgwick.

INVENTOR:

J. M. Dennis  
BY *M. M. & Co.*

ATTORNEYS.

# UNITED STATES PATENT OFFICE.

JAMES M. DENNIS, OF CAMBRIDGE CITY, INDIANA, ASSIGNOR TO HIMSELF  
AND CALEB P. RINKER.

## BRUSH.

SPECIFICATION forming part of Letters Patent No. 240,103, dated April 12, 1881.

Application filed February 18, 1881. (Model.)

*To all whom it may concern:*

Be it known that I, JAMES M. DENNIS, of Cambridge City, in the county of Wayne and State of Indiana, have invented a new and Improved Varnish-Brush, of which the following is a full, clear, and exact description.

Figure 1 is a perspective view of my wooden varnish or paint brush, and Fig. 2 is a sectional view of the same.

10 Similar letters of reference indicate corresponding parts.

The invention consists in the process of separating and preparing woody fiber for varnish or paint brushes, as hereinafter described.

15 In carrying my invention into effect I add to about eight ounces of water two ounces of concentrated alkali and then soak the pieces of wood or bark of suitable size in the boiling solution for about ten minutes, and then I sub-

20 ject the wood or bark to a crushing, pressing, or pounding process, which separates the fibers from each other and from the non-fibrous portion, and then I wash the wood or fibers in clean water, then dry the same. I then boil 25 the pieces of wood in water having a quantity of glue added, for about one-half hour, and finally oil the fibers with olive or other oil to render them elastic.

In making the character of brush shown in 30 the drawings, in which the filamentous portion *a*, the body *b*, and the handle *c* are all formed of a single piece of wood, the piece of wood out of which the brush is to be formed is given the proper shape and outline by turning, shav-

ing, or otherwise, and only the portion *a* is 35 subjected to the treatment above described, and then the wrapper *c* is secured to the body *b*, to prevent breaking and further separating of the fibers by the nails or screws *d*.

Instead of forming the handle *e* of the brush 40 before the treatment for separating the fibers, it is obvious this may be done after such treatment, if desired; and instead of forming the entire brush of a single piece of wood or inner bark, the fibers may be obtained separately by 45 treating, as above described, pieces of the wood or bark of suitable size to make the requisite length of fibers, and subsequently securing the fibers to the handle or body of the brush, by gluing or otherwise, in which case the handle and body may be of any wood or material. 50

Having thus described my invention, I claim as new and desire to secure by Letters Patent—

The process herein described for preparing 55 the fibers of wood in or for the manufacture of brushes, which consists in first soaking the wood in heated alkaline water, then separating the fibers by pressing and pounding, or otherwise, then cleaning the fibers, then boiling the same in agglutinated water, and finally oiling the fibers, substantially as and for the purposes described.

JAMES MONROE DENNIS.

Witnesses:

J. W. POFF,  
E. WILSON.